

April 10, 1956

L. ROGOSIN

2,741,108

FLAME RESISTANT FABRIC

Filed Sept. 20, 1951

Fig. 1.



Fig. 2.



Fig. 4.

INVENTOR

LIONEL ROGOSIN

BY *Rudolph J. Bley*,  
ATTORNEY



Fig. 5

# United States Patent Office

2,741,108

Patented Apr. 10, 1956

1

2,741,108

## FLAME RESISTANT FABRIC

Lionel Rogosin, Weehawken, N. J., assignor to Beaunit Mills, Incorporated, New York, N. Y., a corporation of New York

Application September 20, 1951, Serial No. 247,545

5 Claims. (Cl. 66—194)

This invention relates to novel flame resistant "Orlon" fabrics. More particularly, the invention relates to a novel "Orlon" brushed fabric the flammability of which has been greatly reduced by including in the makeup of the fabric a substantial percentage of saran yarn so that the resulting mixture of saran and "Orlon" yarns in the finished fabric confers a relatively high degree of flame resistance upon the finished fabric.

One of the principal objects of the present invention is to provide a new and improved "Orlon" brushed fabric in which the flammability of the fabric has been greatly reduced by the feature of including in the yarn a substantial percentage of a yarn of relatively low flammability, the presence of which in combination with the "Orlon" yarn imparts a satisfactory degree of flame resistance to the finished fabric.

The manner in which this and other objects and features of the invention are attained will appear more fully from the following description thereof, in which reference is made to typical and preferred procedures in order to indicate more fully the nature of the invention, but without intending to limit the invention thereby.

Referring to the drawing there are shown four views of brushed fabrics illustrating embodiments of this invention.

Fig. 1 is a plan view of a brushed knitted fabric;

Fig. 2 is a side elevation of the brushed knitted fabric shown in Fig. 1;

Fig. 3 is a plan view of a brushed woven fabric; and

Fig. 4 is a side elevation view of the brushed woven fabric shown in Fig. 3.

"Orlon" brushed fabrics are already known to the art, and for certain uses are known to be very desirable. However, for certain other uses where it is necessary to provide fabrics which are relatively flame resistant such as for components of clothing, blankets, etc., for military and civilian personnel where there may be substantial risk from fire hazards, the "Orlon" brushed fabric is unsuitable since it is very highly inflammable. However, since it is otherwise highly desirable for these and other uses, considerable effort has been expended in an effort to confer the necessary degree of flame resistance upon such fabrics. While a great deal of research has been carried out on the flameproofing of fabrics in general, much of this work has taken the direction of treating fabrics and/or the yarns of which the fabrics are composed with chemical agents which are designed to confer the desired flameproofing properties thereon; for example, see A. C. S. Monograph No. 104 entitled "Flameproofing Textile Fabrics" by Robert W. Little, Reinhold Publishing Corporation, 1947. Such procedures, while satisfactory in many cases, are frequently undesirable in that they ordinarily involve a considerable degree of "add-on" of one or more chemical reagents, and this generally alters the hand or other desirable properties of the base fabric in such manner as to detract from its usefulness.

According to the present invention, it has been discovered that if an "Orlon" brushed fabric is made up in

2

such manner as to include a substantial portion of saran yarn during the knitting or other fabrication operation, a finished brushed fabric is obtained that is characterized by a very substantial degree of flame resistance as compared to an otherwise identical brushed fabric without the saran yarn. It is believed that the reason why saran is capable of imparting flame resistance to this brushed fabric is because saran in burning, because of its composition, gives off vapors which tend to extinguished not only its own blaze but that of adjacent inflammable yarns and fibers. Moreover, since the desired flame resistance has been "built in," so to speak, and does not involve the addition to the fabric of chemical flameproofing agents according to flameproofing methods previously known per se in the art, the hand and other desirable characteristics of the finished fabric are not adversely affected as is frequently the case when using chemical flameproofing agents.

In order to indicate still more fully the nature of the present invention the following example of typical procedure is set forth, it being understood that this description is presented by way of illustration only and not as limiting the scope of the invention.

### Example

An "Orlon" fabric was knit on a 20-gauge, 30" cylinder circular Tompkin knitting machine, utilizing 20 stitches for the construction of the back of the fabric.

A backing burl blocked one in and one out was used for laying in yarn on the face of the fabric without distorting the back in any manner.

The yarn employed was as follows:

1 end 20/1 K. P. (cotton karded peeler) for the back;  
1 end 750 denier saran for the face; and 3 ends 200 denier "Orlon" for the face. The ends of "Orlon" and saran yarn to make the face of the fabric were all knitted in one feed.

The yarn percentages were as follows:

|                          | Percent |
|--------------------------|---------|
| 20/1 K. P. -----         | 27.7    |
| 750 denier saran -----   | 40.8    |
| 200 denier "Orlon" ----- | 31.5    |

No dyestuff was applied to the fabric, it being merely boiled off and rinsed. No finish or fire retardants of any kind were applied. The fabric was dried on a vertical pipe drier. The fabric was in circular condition and was then split, after which it was napped six times on a napping machine in conventional manner on a regular rayon setting, and then tentered to 56". This produced a soft pile effect on the face yarn of the fabric.

The saran-Orlon brushed fabric that was produced in the manner described above possessed a soft hand and, more importantly, had acquired a substantial flame resistance in comparison with an otherwise identical "Orlon" brushed fabric containing no saran yarn.

It is to be understood that the novel brushed fabric prepared as described above was made entirely by conventional methods using conventional machines well known in the art.

While the invention has been described more particularly in conjunction with a novel saran-Orlon brushed fabric, it will be understood that saran yarn may be incorporated in other types of brushed fabrics which normally are highly inflammable with similar desirable results, one instance being a saran viscose rayon brushed fabric prepared exactly as described above but with the substitution of viscose rayon yarn for "Orlon" yarn. The fabrics may be woven instead of knitted.

70 It will be appreciated that the saran yarn may be employed in the fabric in varying amounts relative to the "Orlon" or other relatively inflammable yarn without

departing from the spirit of the invention, depending upon the degree of flame resistance desired in the finished fabric.

Although the chemical nature of "Orlon" and saran yarns is well known to those skilled in the art, it may be well to point out that saran is a copolymer of vinylidene chloride and vinyl chloride in which the former predominates—see Fieser and Fieser, "Organic Chemistry," second edition, 1950, page 951, Abernethy Patent No. 2,542,973 and Jones Patent No. 2,543,027. "Orlon" yarn is made from polyacrylonitrile—see Fieser and Fieser, at pages 951-2.

While a specific example illustrating the present invention has been set forth above, it will be apparent that many changes and modifications may be made therein without departing from the spirit of the invention. It is therefore to be understood that the example cited and the particular proportions and details set forth above are intended to be illustrative only and are not intended to limit the scope of the invention.

What is claimed is:

1. A flame resistant brushed fabric comprising a backing prepared from normally inflammable yarn, a facing for said fabric capable of receiving a nap, said facing being constructed from at least two different yarns, at least one of which is highly inflammable in its brushed condition and the other of which comprises saran; said saran being present in substantial amounts determined by the inflammability of the other yarn components comprising said facing, but not less than required to impart flame resistance to said fabric.

2. A fabric as claimed in claim 1 wherein one of the yarns employed in constructing the facing comprises "Orlon."

3. A fabric as claimed in claim 1 wherein one of the yarns employed in constructing the facing comprises rayon.

4. A flame resistant brushed woven fabric comprising a backing prepared from normally inflammable yarn, a

facing for said fabric capable of receiving a nap, said facing being constructed from at least two different yarns, at least one of which is highly inflammable in its brushed condition and the other of which comprises saran, said saran being present in substantial amounts determined by the inflammability of the other yarn components comprising said facing, but not less than required to impart flame resistance to said fabric.

5. A flame resistant brushed knitted fabric comprising a knit cotton backing having attached thereto a facing capable of receiving a nap, said facing being constructed from a combination of "Orlon" and saran yarns, with at least one end of saran yarn being employed per several ends of said "Orlon" yarn, with the number of ends of saran being no greater than required to impart a substantial degree of flame resistance to said fabric.

#### References Cited in the file of this patent

#### UNITED STATES PATENTS

|    |           |                |               |
|----|-----------|----------------|---------------|
| 20 | 290,238   | Johns          | Dec. 18, 1883 |
|    | 599,438   | Bell           | Feb. 22, 1898 |
|    | 668,793   | Bradley        | Feb. 26, 1901 |
|    | 2,019,258 | Holmes         | Oct. 29, 1935 |
|    | 2,156,455 | Kleine         | May 2, 1939   |
|    | 2,239,457 | Gibbons        | Apr. 22, 1941 |
|    | 2,266,631 | Francis        | Dec. 16, 1941 |
|    | 2,279,206 | Randall        | Apr. 7, 1942  |
|    | 2,312,089 | Gobeill        | Feb. 23, 1943 |
|    | 2,313,058 | Francis        | Mar. 9, 1943  |
|    | 2,353,090 | Shelmir et al. | July 4, 1944  |
|    | 2,354,435 | Stedman        | July 25, 1944 |
|    | 2,536,163 | Feild et al.   | Jan. 2, 1951  |
|    | 2,539,301 | Foster         | Jan. 23, 1951 |
|    | 2,585,212 | Backer         | Feb. 12, 1952 |

#### OTHER REFERENCES

Sherman and Sherman: The New Fibers, 1946 (pp. 90, 91).